

# UNITED STATES PATENT OFFICE.

CHARLES STEWART LOUNDS, OF FORT LEE, NEW JERSEY.

## LIQUID COATING COMPOSITION FOR PREVENTING METALLIC SURFACES FROM TARNISHING.

1,146,836.

Specification of Letters Patent. Patented July 13, 1915.

No Drawing.

Application filed March 2, 1915. Serial No. 11,613.

*To all whom it may concern:*

Be it known that I, CHARLES STEWART LOUNDS, of London, England, now residing at Linwood Villa, Edwin avenue, Fort Lee, in the State of New Jersey, have invented a new and useful composition of matter to be used for the purpose of permanently preventing metal surfaces, such as plated silver, brass, copper, gold, silver, nickel, &c., from tarnishing.

The composition consists of the following ingredients combined in the following proportions: celluloid (cuttings) 1 ounce, amyl acetate 80 ounces, oil of cedar  $\frac{1}{2}$  ounce, denatured alcohol 1 ounce.

In mixing the above named composition the celluloid (which is the chief factor) must first be thoroughly dissolved in the amyl acetate, then add the oil of cedar, and denatured alcohol. All of these ingredients must then be thoroughly mingled by agitation.

By the use of the above named composition of matter, either by applying it to the article (to be coated) with a brush, or dip-

ping the article into the liquid you give it a thin coating of celluloid, which prevents the air from tarnishing the article.

My composition of matter is colorless, and waterproof, therefore, after the article has been thoroughly cleaned and coated with the said composition of matter, it will remain untarnished permanently, without having to be cleaned again.

I claim:

1. The herein described composition of matter, consisting of celluloid, amyl acetate, oil of cedar, and denatured alcohol, substantially in the proportions described.

2. The herein composition of matter, for preventing all kinds of plated silver, brass, copper, gold, silver, nickel, and all kinds of metal, from tarnishing, consisting of celluloid 1 ounce, amyl acetate 80 ounces, oil of cedar  $\frac{1}{2}$  ounce, denatured alcohol 1 ounce, substantially as described.

CHARLES STEWART LOUNDS.

Witnesses:

CHAS. BURFEINDT,

SOPHIA M. BURFEINDT.